

A. E. SCHMIDT,  
CHEMICAL MARKER.

APPLICATION FILED OCT. 20, 1919.

1,357,594.

Patented Nov. 2, 1920.

Fig. 1.



Fig. 2.



Fig. 3.



Fig. 4.



INVENTOR:  
Alfred E. Schmidt,

BY  
Russell Everett,  
ATTORNEY.

# UNITED STATES PATENT OFFICE.

ALFRED E. SCHMIDT, OF NEWARK, NEW JERSEY.

## CHEMICAL MARKER.

1,357,594.

Specification of Letters Patent.

Patented Nov. 2, 1920.

Application filed October 20, 1919. Serial No. 331,850.

*To all whom it may concern:*

Be it known that I, ALFRED EDWARD SCHMIDT, a citizen of the United States, and a resident of Newark, in the county of 5 Essex and State of New Jersey, have invented new and useful Improvements in Chemical Markers, of which the following is a specification.

This invention relates in general to a 10 marking device in the nature of a pencil or crayon, and more particularly to a device of this character for marking upon hides, for identification purposes or the like, while the hides are wet from a tanning process.

15 The objects of the invention are to provide a marking composition which chemically acts upon a substance over which the device is drawn to produce a visible inscription in the path of the marking device; to 20 provide a marking device which will produce an indelible and plainly visible inscription; to obtain a marking composition of the character which will produce an inscription or mark which is water proof and will 25 not run or blur; to secure a device which is solid in formation so as to be easily handled; to provide a novel composition of matter for such a marking device; to obtain a marking device comprising a solid composition of 30 matter including a chemical which coacts with another chemical on the substance touched by the marking device, and a vehicle or binder for carrying said chemical; to provide a marking device comprising a 35 solid composition of matter including a chemical and binding ingredients, which is soluble in another chemical, whereby the first-mentioned chemical is liberated from the composition and coacts with said second- 40 mentioned chemical, the binding ingredients then becoming inactive; and to obtain other objects and results as may be brought out by the following description.

45 Referring to the accompanying drawing which illustrates one embodiment of my invention, and in which like numerals of reference indicate the same parts throughout the several views,

50 Figure 1 is a perspective view of one form of stick of my improved marking composition;

55 Fig. 2 is a similar view, showing another form of stick;

Fig. 3 is a perspective view, showing my invention in the form of a pencil, and 55

Fig. 4 is a transverse sectional view through the pencil shown by Fig. 3.

My composition herein described is particularly adapted for placing identification marks on wet hides which have been tanned 60 with vegetable tannin matters. It is the present custom of tanners or leather workers to use a lump of iron sulfate or copperas for marking the hides, which when drawn over a wet hide tanned with vegetable tannin 65 matters produces a black, indelible mark on the hide. However, the lumps of copperas are unwieldy and hard to handle, irregular in shape, and easily crumble.

70 My invention eliminates these difficulties by combining copperas with suitable gelatinous or adhesive binding agents to prevent crumbling and a hardening agent, and molding the composition into any desired form 75 for marking. In making my improved composition I use sulfate of iron (copperas), starch, glue, glucose, and plaster of Paris in the following proportions: 1 pound sulfate iron, 1 ounce starch, 1 ounce glue,  $\frac{1}{2}$  ounce glucose,  $\frac{1}{2}$  ounce plaster of Paris, 80 water.

85 The sulfate of iron is dissolved in one quart of water, to which is added the starch dissolved in two ounces of water, the glue dissolved in two ounces of water, the glucose dissolved in one ounce of water, and the plaster of Paris. These ingredients are thoroughly mixed together, and the whole mass boiled while stirring, until the compound acquires a consistency which will 90 solidify when cooled. The compound is then poured while hot into any suitable mold and allowed to cool and solidify.

95 Obviously, the compound can be molded into many shapes suitable for marking, such as the flat rectangular stick 1 shown by Fig. 1, or the cylindrical stick 2 shown by Fig. 2. If desired the sticks 1 or 2 can be covered, as by gluing between two pieces of wood, or the like, 3 and 4, so that the compound can be handled without soiling the hands, and will be protected from being acted upon by other chemicals. The marking device is thus in the form of a pencil 5, which can be sharpened in the conventional 100 manner, as at 6, to expose the compound for 105

marking. The marking device is used similarly to a conventional pencil or crayon, and when drawn over a wet hide which has been tanned with vegetable tannin matters, the compound slightly dissolves and liberates the copperas, which chemically coacts with the chemicals used in the tanning process to produce an indelible, clear, and unblurrable black mark, the binding and hardening agents passing off inactive.

Other chemicals than copperas or the sulfate of iron can be utilized, and for marking on wet hides any iron salt is equally well adapted as the sulfate of iron. Furthermore, I could use other binding agents than the starch, glue and glucose, for instance, casein, gum, or sugar; and, as a hardening agent, I could use chalk, or a carbonate of lime, instead of the plaster of Paris. However, the plaster of Paris is preferable in my present compound, as it is firmer.

Having thus described the invention, what I claim is:

1. A marking composition comprising a substance chemically coactive with the surface of a tanned hide, and binding and hardening agents.

2. A marking composition comprising a

substance chemically coactive with the wet surface of a hide in the process of tanning, and binding and hardening agents.

3. A marking composition comprising a substance chemically coactive with the surface of a wet hide tanned in vegetable tannin matter, and binding and hardening agents.

4. A marking composition comprising an iron salt, and binding and hardening agents.

5. A marking composition comprising an iron salt, a gelatinous substance, and a hardening agent.

6. A marking composition comprising an iron salt, a binding agent, and plaster of Paris for hardening.

7. A marking composition comprising an iron salt, starch, glue, glucose, and a hardening agent.

8. A marking composition comprising an iron salt, starch, glue, glucose, and plaster of Paris.

9. A marking composition comprising one pound of an iron salt, one ounce of starch, one ounce of glue, one-half ounce of glucose, and one-half pound of plaster of Paris.

ALFRED E. SCHMIDT.